

# United States Patent

[11] 3,590,998

[72] Inventors **David J. Collins**  
Walnut Creek;  
Guy H. Harris, Concord, both of, Calif.  
[21] Appl. No. **796,158**  
[22] Filed **Feb. 3, 1969**  
[45] Patented **July 6, 1971**  
[73] Assignee **The Dow Chemical Company**  
Midland, Mich.

3,290,351 12/1966 McKay ..... 260/455  
2,835,625 5/1958 Lo ..... 260/455 X

## FOREIGN PATENTS

750,568 6/1956 Great Britain ..... 260/455  
1,179,312 12/1958 France ..... 260/455

Primary Examiner—Frank W. Lutter  
Assistant Examiner—Robert Halper  
Attorneys—Griswold and Burdick, Bruce M. Kanuch and  
William R. Norris

## [54] FLOTATION OF SULFIDE ORES 6 Claims, No Drawings

[52] U.S. Cl. ..... 209/166,  
260/455  
[51] Int. Cl. ..... B03d 1/02,  
C07c 153/07  
[50] Field of Search ..... 209/166,  
167, 252/61; 260/455

## [56] References Cited

### UNITED STATES PATENTS

|           |         |               |           |
|-----------|---------|---------------|-----------|
| 1,640,218 | 8/1927  | Sayre.....    | 209/166   |
| 1,674,166 | 6/1928  | Douglass..... | 209/166   |
| 2,691,635 | 10/1954 | Harris.....   | 209/166 X |
| 3,012,053 | 12/1961 | Lesslie.....  | 260/455   |
| 3,224,863 | 12/1965 | D'amico.....  | 260/455 X |

**ABSTRACT:** An improvement in the concentration of ores by flotation which comprises subjecting a sulfide ore in the form of a pulp to a flotation process in the presence of an effective quantity of a flotation collector comprising a compound corresponding to the formula



wherein R and R<sub>2</sub> are hydrocarbon groups and R<sub>1</sub> is an alkylene group. Certain of the indicated compounds provide enhanced recovery of and/or selectivity of sulfide minerals of Cu, Zn, Mo, Co, Ni, Pb and As over iron sulfide.

## FLOTATION OF SULFIDE ORES

## BACKGROUND

Flotation is a process of treating a mixture of finely divided mineral solids, e.g., a pulverulent ore, suspended in a liquid whereby a portion of such solids are separated from other finely divided mineral solids by introducing a gas (or providing a gas *in situ*) into the liquid to produce a frothy mass containing certain desired solids on the top of the liquid, and leaving suspended (unfrothed) solids in the liquid.

Flotation is based on the principle that introducing a gas into a liquid containing solid particles of different materials suspended therein causes adherence of some gas to certain suspended solids and not to others and makes the particles having the gas thus adhered thereto lighter than the liquid. Accordingly, they rise to the top of the liquid to form a froth.

Various flotation agents have been admixed with the suspension to improve the frothing process. Such added agents are classed according to the function to be performed: collectors, e.g., high carbon chain compounds such as collectors for sulfide minerals including xanthates, thionocarbamates, and the like; frothers which impart the property of forming a stable froth, e.g., natural oils such as pine oil and eucalyptus oil; modifiers such as activators to induce flotation in the presence of a collector, e.g., copper sulfate; depressants, e.g., sodium cyanide, which tend to prevent a collector from functioning as such on a mineral which it is desired to retain in the liquid, and thereby discourage a substance from being carried up and forming a part of the froth; pH regulators to produce optimum metallurgical results, e.g., lime, soda ash and the like.

It is of importance to bear in mind that additaments of the above type are selected for use according to the nature of the ore, the mineral sought to be recovered, and the other additaments which are to be used in combination therewith.

An understanding of the phenomena which makes flotation a particularly valuable industrial operation is not essential to the practice of the present invention. They appear, however, to be largely associated with selective affinity of the surface of particulated solids, suspended in a liquid containing entrapped gas, for the liquid on one hand, the gas on the other.

The flotation principle is applied in a number of mineral separation processes among which is the selective separation of such minerals as sulfide copper minerals, sulfide zinc minerals, sulfide molybdenum minerals and others from sulfide iron minerals. The present invention concerns the use of a unique class of compounds as collection agents in a flotation process. With some of these collectors better recoveries are realized and with others improved selectivity is achieved. Certain of these agents produce improvement in both aspects.

## SUMMARY

The present invention concerns an improved method of flotation separation of sulfide minerals which comprises subjecting a sulfide ore to a flotation process in the presence of a compound corresponding to the formula



wherein R is a hydrocarbyl group, other than an aryl or alkaryl; R<sub>1</sub> is an alkylene group, and R<sub>2</sub> is a hydrocarbyl group other than aryl or alkaryl; said compounds acting as flotation collectors in the concentration of sulfide minerals of copper, zinc, molybdenum, cobalt, nickel, lead, arsenic and others from ores in preference to other minerals.

## PREFERRED EMBODIMENTS

In the practice of the present invention the present compounds are employed as flotation collectors using standard flotation techniques. Preferable compounds correspond to the formula



5 wherein R represents a hydrocarbyl group selected from the group consisting of a branched or straight chain alkyl or alkenyl group or an cycloalkyl or cycloalkenyl group, preferably containing from 1 to 10 carbon atoms, or an aralkyl group; R<sub>1</sub> represents an alkylene group, preferably containing from 1 to 10 carbon atoms, and R<sub>2</sub> represents a hydrocarbyl group selected from the group consisting of an alkyl, alkenyl, cycloalkyl or cycloalkenyl group, preferably containing from 1 to 8 carbon atoms, an aralkyl or aralkenyl group.

10 The flotation collector compounds as defined herein can be prepared by the interaction of an ester of a primary amino acid with a compound corresponding to the general formula



20

wherein M represents a metal cation and R<sub>2</sub> is the same as defined hereinbefore, the desired product being obtained with coformation of the metal acetate through cleavage of the



25

bond.

30 The flotation collector compounds as defined herein are particularly suitable for use in standard flotation processes to concentrate copper sulfide and other like minerals from sulfide ores. In such processes, a pulp is first prepared by wet grinding the ore to a suitable size with or without a pH modifier. A suitable frothing agent is then added, e.g., pine oil, cresylic acid, polyalkoxyparaffin and the like. An effective quantity of the flotation collector compound as defined herein is then added usually ranging from about 0.01 lb. to about 0.25 lb. per ton of pulp and the pulp usually agitated and aerated. The copper sulfide minerals and other like sulfide minerals, except iron sulfide, collect as a froth which is readily overflowed or skimmed off from the residual gangue and other nondesired materials and the metal values therein recovered.

35 The following Examples will facilitate a more complete understanding of the present invention but they are not meant to limit the scope of the invention to the specific embodiments incorporated therein.

55

## EXAMPLE 1

Various species of flotation collector compounds within the scope of the present invention were employed in the flotation recovery of copper from a sulfide ore obtained from Southwestern United States employing the following procedure. A sample of ore was ground for 4 minutes at a pulp density of 64.5 percent by weight solids with 2.0 lbs./ton of lime. The pulp was then conditioned for 2 minutes at a pH of 10.3 with a collector compound and 0.05 lbs./ton of a frother. The pulp was then floated for 4 minutes. A standard flotation collector compound consisting of a thionocarbamate compound corresponding to the formula



70

75 was employed as a control. The specific collector compounds, concentrations of collectors, and analysis of the concentrates and tailings for copper are set forth in the following Table I.



